

June 4, 1929.

G. W. ELMEN

1,715,647

MAGNETIC MATERIAL

Filed June 30, 1926

6 Sheets-Sheet 1



Inventor:  
Gustaf W. Elmen

by W. Griggs

Atty.

June 4, 1929.

G. W. ELMEN

1,715,647

MAGNETIC MATERIAL

Filed June 30, 1926

6 Sheets-Sheet 2



Inventor:  
Gustaf W. Elmen

by E. W. Griggs

Att'y.

June 4, 1929.

G. W. ELMEN

1,715,647

MAGNETIC MATERIAL

Filed June 30, 1926

6 Sheets-Sheet 3

Fig.10



Fig.11



Fig.13



Fig.12



Fig.14



Inventor:  
Gustaf W. Elmen

by W. Briggs

Atty

June 4, 1929.

G. W. ELMEN

1,715,647

MAGNETIC MATERIAL

Filed June 30, 1926

6 Sheets-Sheet 4

Fig.15



Fig.17



Fig.16



Fig.18



Inventor:  
Gustaf W. Elmen

by *W. Elmen* Att'y.

June 4, 1929.

G. W. ELMEN

1,715,647

MAGNETIC MATERIAL

Filed June 30, 1926

6 Sheets-Sheet 5



Fig. 19



Fig. 20



Fig. 21



Fig. 22

Inventor:  
Gustaf W. Elmen

by *E. Griggs*

Atty.

June 4, 1929.

G. W. ELMEN

1,715,647

MAGNETIC MATERIAL

Filed June 30, 1926

6 Sheets-Sheet 6



Fig. 25



Fig. 26



Fig. 27



Fig. 28



Inventor:  
Gustaf W. Elmen

by

W. Briggs

Atty.

## UNITED STATES PATENT OFFICE.

GUSTAF W. ELMEN, OF LEONIA, NEW JERSEY, ASSIGNOR TO WESTERN ELECTRIC COMPANY, INCORPORATED, OF NEW YORK, N. Y., A CORPORATION OF NEW YORK.

## MAGNETIC MATERIAL.

Application filed June 30, 1926. Serial No. 119,623.

This invention relates to magnetic materials and more especially to magnetic alloys containing nickel, cobalt, and iron. The particular proportions of the several 5 constituents and the methods of preparation of the material are set forth hereinafter.

There have hitherto been described magnetic alloys exhibiting relatively constant permeability over a range of magnetizing 10 forces and also exhibiting relatively low hysteresis loss. Such a material is described in French Patent No. 606,649 granted March 12, 1926. There have also been known 15 magnetic materials comprising nickel and iron and containing a very small amount of cobalt as an impurity. An example of such an alloy is that described in the paper by Arnold and Elmen entitled "Permalloy" published in the Journal of the Franklin 20 Institute for May, 1923, volume 195, pages 621 to 632.

The present invention relates to magnetic materials exhibiting constancy of permeability of an entirely different order than 25 that of the material described in the French patent. It relates, moreover, to compositions in which the cobalt content is in excess of the slight amounts which ordinarily would be present as a result of using good 30 commercial nickel and is sufficient, when the alloy is given the proper heat treatment, to impart thereto properties not characteristic of previously-known magnetic materials.

A novel and striking property of magnetic 35 materials in accordance with this invention resides in their extraordinarily constant permeability over a considerable range of flux densities extending from zero upward.

Another important property is substantially complete absence of hysteresis over a considerable range of flux densities from zero upward.

Another property is the relatively high 45 initial permeability and high permeability throughout the range of flux densities utilized in magnetic materials for telephone, telegraph and cable circuits and apparatus.

At higher flux densities the hysteresis loss, 50 the remanence, and the coercive force are low.

At still higher flux densities the hysteresis

loop widens out and assumes a peculiar form, characterized by a constriction at the origin.

55

The resistivity of magnetic materials in accordance with this invention compares favorably with that of other magnetic materials and can be controlled by varying the proportions of nickel, cobalt and iron or by 60 the addition of a fourth element.

The characteristics of constancy of permeability and negligible hysteresis loss which are exhibited by these new materials in the range of flux densities from zero to 900 65 c. g. s. units, more or less, are important in signaling and other applications in which uniformity of characteristics over a wide working range is demanded. The resulting advantages of reduced energy dissipation 70 and reduction of wave distortion will be apparent to those skilled in the signaling art. However, these materials exhibit many desirable properties at high field strengths and hence are useful for general application as 75 electromagnetic materials. In particular the low hysteresis, low remanence, low coercivity, and relatively high specific resistance are noteworthy.

A particular magnetic material in accordance 80 with the invention consists of approximately 45% nickel, 25% cobalt and 30% iron with about .5% of manganese added to increase the workability. This material may be hot annealed and cooled slowly in the furnace in accordance with the first heat treatment hereinafter specified. It has a face-centered cubic crystalline structure. The curves given in Figs. 1 to 9, inclusive, relate 85 to a specimen of this particular composition but are illustrative of the properties of other compositions within the scope of the invention.

Some of the properties of this particular material, when prepared as hereinafter 90 stated, are illustrated in Figs. 1 to 9, inclusive of the accompanying drawings, in which:

Fig. 1 shows a magnetization curve;

Fig. 2 is a curve illustrating the relation 100 of permeability to magnetizing force over a range of magnetizing forces up to nine gauss.

Fig. 3 shows half of a hysteresis loop of

this material as compared with hysteresis loops for Armco iron and silicon steel under similar conditions, "a" indicating the new material, "b" silicon steel, and "c" Armco iron.

Figs. 4 to 8, inclusive, show in each case half of a hysteresis loop at different magnetizing forces respectively; and

Fig. 9 shows half of a hysteresis loop of the material at a considerably higher maximum flux density than in the preceding figures.

Figs. 10 to 14, inclusive, illustrate the properties of a specimen of material of approximately 60% nickel, 15% cobalt and 25% iron; Fig. 10 shows both a magnetization curve and a hysteresis loop for  $B=13250$ ; Fig. 11 is a graph of permeability for varying values of magnetizing force; and Figs. 12 to 14, inclusive, are halves of hysteresis loops for several values of induction; Figs. 13 and 14 also show the magnetization curve of the virgin material as well as the hysteresis loops.

Figs. 15 to 18, inclusive, illustrate the properties of a composition of approximately 73.8% nickel, 6% cobalt, 20.5% iron and .2% manganese; Fig. 15 is a graph of permeability with varying values of magnetizing force; and Figs. 16 to 18 illustrate halves of hysteresis loops for several values of induction.

Figs. 19 to 22, inclusive, relate to a material comprising approximately 50% nickel, 30% cobalt and 20% iron; Fig. 19 is a graph of permeability for varying values of magnetizing force; and Figs. 20 to 22 are halves of hysteresis loops for several different values of maximum induction.

Figs. 23, 24, 25, 26, 27 and 28 relate to a composition of approximately 10% nickel, 70% cobalt and 20% iron with a small fraction of 1% of manganese; Fig. 23 is a graph of permeability with varying values of magnetizing force; Fig. 24 shows a half hysteresis loop for an applied magnetizing force of 80 gauss and also a magnetization curve of the virgin material which curve is distinguished from the loop by having dots instead of circles; and Figs. 25 to 28 illustrate halves of hysteresis loops for varying values of maximum induction.

In all the figures of the drawing which involve magnetizing forces and flux densities these quantities are plotted in c. g. s. units.

The curves of Figs. 1 and 2 indicate the remarkable constancy of permeability up to a magnetizing force of almost two gauss. In accordance with Fig. 2 the initial permeability is about 460 for this particular material. The curve of Fig. 1 also shows that the material has the high flux density of 15000 c. g. s. units at a magnetizing force of 45 gauss.

Curve "a" of Fig. 3 represents the upper

half of the hysteresis loop for this alloy for flux densities up to 600 c. g. s. units represented as a straight line. By ballistic methods no hysteresis loss could be detected and the coercive force and remanence were indicated as zero. By more accurate inductance bridge methods, applicable to low inductions, the hysteresis loss was found to be  $.024 \times 10^{-3}$  ergs per cu. cm. per cycle at an induction of 100 c. g. s. units. This value is so nearly negligible that the hysteresis loss could not be represented on any feasible scale that could be used in the drawings and hence the hysteresis loop appears as a straight line.

The hysteresis loss in a nickel-iron alloy containing 78½% nickel and 21½% iron, heat treated to develop high initial permeability, is much less than for silicon steel or iron. In a particular sample of such an alloy, the hysteresis loss at an induction of 100 c. g. s. units was found to be  $33 \times 10^{-3}$  ergs per cu. cm. per cycle, which is over 1000 times that found by the inductance bridge method for the specimen composed of 45% Ni, 25% Co, and 30% Fe.

Figs. 4 to 9, inclusive, illustrate half hysteresis loops of the material for various maximum inductions and show the manner of growth of the hysteresis loss with increasing induction. The curve of Fig. 4 is similar to the curve "a" of Fig. 3, the circles on this graph indicating the ascending branch and the dots the descending branch. The dots and circles fall on a straight line passing through the origin, indicating the absence of hysteresis, remanence and coercive force. The magnetizing force and maximum induction under which this remarkable condition prevails are the same as those for constancy of permeability. Fig. 4 indicates that the magnetic material has an entirely negligible change of permeability up to inductions of 600 c. g. s. units.

Figs. 5 to 8, inclusive, show the growth of the hysteresis loss as the flux density increases above the highest value shown in Fig. 4. Appearance of hysteresis is evident in Figs. 5 and 6, for example, but the areas of the loops are comparatively small and the hysteresis loss is not material. When the flux density reaches values of 1500 or more, as shown in Figs. 7 and 8, the hysteresis loss increases rapidly but it is to be noted that the residual magnetization and the coercive force are still practically zero.

Fig. 9 shows half of the hysteresis loop for a flux density of approximately 15,000 c. g. s. units. This loop has the general shape of the ordinary hysteresis loop obtained with iron and other magnetic materials. It differs radically from the curves of Figs. 7 and 8 in that the coercive force and remanence are considerable although less than in most magnetic materials. This

is particularly true of the remanence. The hysteresis loss at this high maximum flux density is also relatively small compared with that of other magnetic materials.

5 The curves of Figs. 10 to 14, inclusive, relate to a composition consisting of approximately 60% nickel, 15% cobalt and 25% iron. In this case the initial permeability is 631 and no change of permeability 10 appears up to a flux density of 700 c. g. s. units.

A composition consisting of approximately 70% nickel, 15% cobalt and 15% iron has an initial permeability of 390 and no appreciable 15 change in permeability up to inductions of 200 c. g. s. units.

The curves of Figs. 15 to 18, inclusive, relate to a composition consisting of approximately 73.3% nickel, 6% cobalt and 20.5% 20 iron and .2% manganese which has an initial permeability of 1430 and no appreciable change in permeability up to inductions of 715 c. g. s. units. The maximum permeability is about 5600 at a magnetizing force of 25 1.1 gauss.

A composition of approximately 20% nickel, 50% cobalt and 30% iron exhibits a negligible change of permeability at magnetizing forces of 4 gauss which produce in 30 this instance a flux density of 450 c. g. s. units.

The curves of Figs. 19 to 22, inclusive, relate to a composition of approximately 50% nickel, 30% cobalt and 20% iron which possesses 35 an initial permeability of 231 which is constant up to value of  $B=716$  or  $H=3.1$ .

Figs. 23 to 28, inclusive, relate to a composition of 10% nickel, 70% cobalt and 20% iron which has constant permeability and 40 zero hysteresis loss up to a flux density of 225, the permeability being 57 in this range.

It will be noted that the iron content ranges between 10% and 40% in all of these 45 compositions. Such compositions have small or entirely negligible hysteresis loss for values of  $B$  up to 500 or 1000 as well as negligible coercive force and remanence at inductions of 500 to 1000 and very low coercive force and remanence, often approaching 50 zero, at inductions up to 5000 c. g. s. units.

The range of proportions of the materials, nickel, cobalt and iron, may be stated in general as follows: The magnetic material contains nickel in a substantial percentage of the total nickel, cobalt and iron content; cobalt in a percentage whose lower limit is a few percent, and of an upper limit of considerably more than one-half the material, and the balance iron. For the highest 55 values of initial permeability combined with constancy of permeability experiments have indicated that the nickel should comprise at least 20% of the magnetic material content.

The highest degree of constancy of permeability combined with high initial permea-

bility and low hysteresis loss has been obtained with percentages of iron ranging up to 40% although percentages of iron somewhat above 40% yield materials having to some extent the desirable properties herein 70 described.

In order to further illustrate the properties of these materials the following additional data is given. The composition of 45% nickel, 25% cobalt, and 30% iron, hereinbefore described, has a resistivity of 19 micro-ohm-cms.; a maximum permeability of 2075 at  $H=4.12$ ; remanence of 3400 and coercive force of 1.3 after the application of a magnetizing force of  $H=50$  gauss. The 75 hysteresis loss is negligible at a maximum flux density of 570 c. g. s. units, and is 9.54 ergs per cu. cm. per cycle at 820, 15.65 ergs at 960, 93.2 ergs at 1500, 1185 ergs at 5050, 2500 ergs at 8480, and 3375 ergs at 14900. 85

The material comprising 60% nickel, 15% cobalt and 25% iron has a flux density of 13,250 c. g. s. units at  $H=30.7$ ; a resistivity of 17.5 micro-ohm-cms., remanence and coercive force of 1700 and .7 respectively after 90 an applied field of  $H=30.7$  gauss and a maximum permeability of 2680 at  $H=2.45$ . The hysteresis loss is negligible up to  $B=695$ , and is 1.24 ergs per cu. cm. per cycle at a maximum flux density of 725 c. g. s. units, 95 8.4 ergs at 840, 27 ergs at 1050, 88 ergs at 1520, 632 ergs at 5400, 1240 ergs at 8230, and 1508 ergs at 13,250.

The material of 73.3% nickel, 6% cobalt, 20.5% iron and .2% manganese has a resistivity of 15.5 micro-ohm-cms.; remanence and coercive force of 2700 and .35 respectively after an applied magnetizing force of  $H=21$  gauss; maximum permeability of 5600 at  $H=1.1$  gauss; and negligible hysteresis loss at flux densities up to 715 c. g. s. units. The hysteresis loss per cu. cm. per cycle is 23 ergs at a flux density of 1520 c. g. s. units, 348 ergs at 5125, and 783 ergs at 11,500. 105

The material of 10% nickel, 70% cobalt, and 20% iron with a fraction of 1% of manganese has a resistivity of 15.36 micro-ohm-cms.; remanence and coercive force of 9340 and 3.56 after an applied magnetizing force 115 of 80 gauss; maximum permeability of 1545 at  $H=6.5$ ; and negligible hysteresis loss at flux densities up to 228 c. g. s. units. The hysteresis loss per cu. cm. per cycle is 8 ergs at a flux density of 340 c. g. s. units, 150 ergs at 620, 1040 ergs at 1700, 2740 ergs at 3950, and 14,160 ergs at 15,500 c. g. s. units. 120

In each case the remanence and coercive force are negligible at flux densities at which the permeability is constant and the hysteresis loss negligible, and small at higher values of flux density. The tendency of the remanence and coercivity to remain small after the application of magnetizing forces 125 higher than those at which the permeability 130

remains constant is indicated in the drawings. For example in Fig. 8 the coercive force and remanence are indicated as zero after an applied magnetizing force of 3.2 5 gauss and a flux density of over 5,000 c. g. s. units.

Any of the compositions above indicated 10 may include small quantities of manganese, either as an impurity or added to make the material more workable. Chromium or similar elements or substances may be added to increase the specific resistance of the material or for other purposes.

A peculiar characteristic, often exhibited 15 by magnetic materials in accordance with the invention, is that the application of a direct current or uni-directional magnetizing force of large value and its subsequent reduction to a low value causes the substance 20 to have a greatly increased permeability for superimposed low alternating magnetizing forces. In a particular case the application of a large uni-directional magnetizing force of about 25 gauss to the composition of 25 45% nickel, 25% cobalt and 30% iron and its subsequent removal increases the initial permeability from 435 to 750.

In other words, the permeability curve 30 follows the curve of Fig. 2 for increasing applied magnetizing fields but on decreasing the field by small steps and remeasuring the permeability the values of permeability depart from the curve of Fig. 2. This departure is not great until the point of maximum 35 permeability is reached. To the left of the point of maximum permeability, the value of permeability, after high magnetization, is considerably above the curve, and, in the 40 particular case mentioned above, had an initial value of 750. When a specimen of material is thus highly magnetized the characteristic of constant permeability for a range of magnetizing forces is impaired. To bring the initial permeability back to 45 a lower value it is necessary to demagnetize the material. To restore the constancy of permeability to the fullest extent it is advisable to give the material a renewed heat treatment.

50 Another characteristic usually exhibited by these materials is that the magnetization curve often lies partly without the hysteresis loop for high values of induction. A typical case is indicated by Fig. 10 where 55 the magnetization curve (indicated by dots) is shown crossing the lower branch of the hysteresis loop (indicated by small circles) at an induction of  $B=$ about 500 and joining it again at an induction of  $B=$ about 7000. 60 In Fig. 13 the magnetization curve lies wholly within the hysteresis loop and in Fig. 14 is shown the case where the magnetization curve crosses and has a small portion lying without the hysteresis loop. For all 65 hysteresis loops of this particular specimen

for maximum inductions greater than shown in Fig. 14 the magnetization curve has a portion lying without the hysteresis loop.

Another characteristic is that the hysteresis loss reaches a maximum at a certain 70 value of flux density and does not increase for greater flux densities.

The magnetic properties of materials in accordance with this invention are subject 75 to change under the influence of mechanical strains and stresses and consequently due precautions must be taken in their utilization to avoid excessive strains and stresses.

Magnetic materials, in accordance with 80 this invention, may be prepared by melting the constituents together in an induction furnace. Good grades of material of commercial purity are suitable. The molten metal is cast into rods or bars. These rods or bars are worked by rolling, swaging, or 85 drawing into desired shapes.

After the mechanical fabrication of the parts into their final shapes they are heat treated in order to produce the desired magnetic properties. The temperature to which 90 the material is heated and the rate of cooling determine very largely the relative values of the several magnetic characteristics.

For heat treatment as hereinafter described about 40 grams of the material is 95 prepared in the form of a thin tape which is rolled into a flat spiral. The thickness of the spiral i. e. the width of the tape is 1/8 inch (3.175 mm.). The internal diameter of the spiral is 3 inches (7.62 cm.) 100 and the external diameter 3-1/2 inches (8.89 cm.).

In accordance with a first method of preparation, the material may be pot annealed, using ordinary precautions to prevent oxidation, at about 1100° C. for at 105 least one hour, after which it is allowed to cool slowly to room temperature in the furnace. This is the method which was used in production of the materials, whose 110 magnetic characteristics are shown in Figs. 1 to 28, inclusive.

In a particular instance in which this first method was used the material was placed in a nichrome pot. The pot was 115 about 1/2 full. A rim around the pot projected above the cover. A layer of iron filings, placed on the cover, was retained by the rim. The pot was placed in an electric furnace when its temperature was about 120 900° C. In 90 minutes the temperature of the pot rose to 1100° C. and it was maintained at that temperature for 70 minutes. The material was then allowed to cool in the furnace and reached a temperature of 350° 125 C. in 180 minutes of cooling time.

In accordance with a second method the pot annealed material is reheated above the magnetic transition temperature i. e., about 725° C. and cooled faster than in the first 130

case, for example, at about an average rate of 2° C. to 5° C. per second down to about 350° C. and thereafter to room temperature at any desired rate.

5 In accordance with a third method the pot annealed material is reheated to about 725° C. and is cooled rapidly as, for example, by placing the spiral of tape weighing 40 grams on a large copper plate in the 10 open air. The 40 grams of material is in the form of thin tape wound into a spiral ring of internal diameter 3 inches (7.62 cm.), external diameter 3-1/2 inches (8.89 cm.), and thickness 1/8 inch (3.175 mm.), 15 which is the width of the tape.

Of these methods the first gives the materials the most nearly constant permeability and the lowest hysteresis loss over a wide range of field strengths.

20 Treatment in accordance with the second method gives higher permeability, particularly at low magnetizing forces but the permeability is not so constant or not constant over so great a range.

25 The third method produces still higher permeability particularly in compositions with a high nickel content but with a greater tendency to variations in permeability with increasing magnetizing forces and greater 30 tendency to increase in hysteresis loss at low field strengths.

The methods of heat treatment may be varied as experience may indicate. The particular methods given illustrate the principle that the degree in which the various properties are present is dependent to some extent upon the heat treatment and that various special properties may be obtained to an increased extent not only by proper 40 selection of the proportions of the constituents of the composition but also by selecting a suitable heat treatment.

Among the uses for which this material is adapted are coil or lumped loading and 45 continuous loading of low and carrier frequency signaling conductors in submarine and land line telephony and telegraphy, loading coils for composite telephone and telegraph systems, repeating coils or trans- 50 formers, especially battery supply coils, wave filter coils, certain important classes of relays, dynamo-electric machinery, high frequency electromagnetic devices, and magnetic circuits of electrical measuring instru- 55 ments.

As an illustration of uses of magnetic materials in accordance with the present invention in order to take advantage of the important characteristic of constant permeability over a range of magnetizing forces, 60 may be mentioned its use for the continuous loading of telephone conductors in accordance with applicant's United States Patent 1,586,883 granted June 1, 1926, or the 65 continuous loading of long submarine tele-

graph cables for high speed signaling in accordance with United States patent to Buckley 1,586,874 granted June 1, 1926. The use of the present material offers great advantages over the use of materials of 70 permeability variable within the range of magnetizing forces employed.

The magnetic material of a continuously loaded conductor may be given the desired magnetic properties by first applying the 75 loading material to the conductor and then heat treating a coil of the conductor of considerable radius in a suitably large furnace in accordance with the methods hereinbefore described. 80

What is claimed is:

1. A magnetic material including at least two magnetic elements and having negligible variation in permeability over a range of flux densities at least 50 c. g. s. units in 85 width and lying between zero as a lower limit and 5000 c. g. s. units as an upper limit.

2. A magnetic material including at least two elements of the magnetic group having negligible hysteresis loss over a range of 90 flux densities of at least 50 c. g. s. units and lying within the range employed in electric communication circuits.

3. A magnetic material including at least two elements of the magnetic group, having 95 substantially constant permeability for flux densities below the general range of B=500 to 1000.

4. A magnetic material including at least two elements of the magnetic group having 100 negligible hysteresis loss for flux densities below the general range of B=500 to 1000.

5. A magnetic material comprising nickel 10% or more, cobalt 5% or more, and iron in a substantial amount but not to exceed 105 about 45%, the nickel-cobalt-iron content being at least 85% of the total.

6. A magnetic material having a variation in permeability of less than 2% over a range of flux densities from zero to at least 50 110 c. g. s. units.

7. A magnetic material having a variation in permeability of less than 2% for flux densities up to at least 600 c. g. s. units.

8. A magnetic composition having a 115 hysteresis loss of less than  $.15 \times 10^{-3}$  ergs per cycle per cubic centimeter for a range of magnetizing forces from zero up to at least 50 c. g. s. units.

9. A magnetic material having negligible 120 variation in permeability over a wide range of flux densities which requires the application of a reverse magnetizing force a few tenths of a c. g. s. unit or less to restore the flux to zero after the application of a magnetizing force sufficient to produce a value of induction up to B=5000. 125

10. A magnetic material having negligible variation in permeability over a wide range of flux densities and having a residual flux 130

- of less than a few hundred c. g. s. units after the application of a magnetizing force sufficient to produce flux densities up to  $B=5000$ .
11. A magnetic material containing cobalt and having substantially constant permeability over a range of low magnetizing forces from zero to at least  $\frac{1}{2}$  c. g. s. unit.
12. A magnetic composition comprising nickel, cobalt and iron as essential elements thereof characterized in that it forms part at least of a magnetic circuit in inductive relation to an electric conductor.
13. A magnetic material having negligible variation in permeability over the general range of flux densities below  $B=500$  to 1000 c. g. s. units comprising nickel, cobalt and iron.
14. A magnetic composition comprising nickel, cobalt and iron as essential constituents thereof characterized in that the composition has been heat treated to give it a constant permeability over a range of low magnetizing forces extending from zero to at least  $\frac{1}{2}$  c. g. s. unit.
15. A magnetic composition comprising nickel, cobalt and iron as essential elements thereof characterized in that it has lower hysteresis loss at all inductions than Armco iron.
16. A magnetic composition containing nickel, cobalt and iron having negligible hysteresis loss for values of induction up to at least 500 c. g. s. units.
17. A magnetic composition containing nickel, cobalt and iron as essential constituents thereof having a coercive force of a few tenths of a c. g. s. unit or less for values of induction up to at least 5000 c. g. s. units.
18. A magnetic material having negligible variation in permeability over a wide range of flux densities, comprising nickel, cobalt and iron, in which a magnetizing force of 45 gauss induces a flux of 15,000 c. g. s. units or more.
19. A magnetic composition comprising nickel, cobalt and iron as essential elements thereof characterized in that the hysteresis loss increases very rapidly over a small range of increasing magnetizing forces while for smaller forces the hysteresis loss is negligible.
20. A magnetic composition comprising nickel, cobalt and iron as essential constituents thereof characterized in that the composition has been heat treated to give a constant permeability over a wide range of low magnetizing forces and further characterized in that the permeability is substantially constant at magnetizing forces from zero to at least around one gauss.
21. A magnetic composition comprising as essential constituents thereof nickel, cobalt and iron having substantially constant permeability and substantially no hysteresis, remanence, or coercivity for a range of low magnetizing forces; variable permeability, appreciable hysteresis and substantially no remanence or coercivity for forces within a higher range; and increasing remanence and coercivity for increasing forces above the latter range.
22. A magnetic material, comprising as essential constituents thereof nickel, cobalt and iron, having substantially constant permeability at magnetizing forces from zero upward to a certain value and having at larger magnetizing forces a considerably higher permeability, which is retained after a very large magnetizing force is applied and removed.
23. A magnetic material containing nickel, cobalt and iron as essential constituents thereof characterized in that the reversible permeability possessed by the material at low unidirectional magnetizing forces is increased to a higher value by the application and removal of a large magnetizing force.
24. A magnetic material comprising nickel, cobalt and iron in which the cobalt content comprises approximately 10% to 35% of the nickel-cobalt-iron content.
25. A magnetic composition comprising nickel, cobalt and iron as essential elements thereof characterized in that iron constitutes around 50% or less of the nickel-cobalt-iron content.
26. A magnetic composition comprising nickel, cobalt and iron as essential elements thereof characterized in that the iron comprises around 50% or less and the cobalt around 35% or less of the nickel-cobalt-iron composition.
27. A magnetic material comprising nickel, cobalt and iron as essential constituents thereof in which the nickel component comprises 9% to 81% of the nickel-cobalt-iron content.
28. A magnetic material comprising nickel, cobalt and iron as essential constituents thereof in which the nickel component comprises 30% to 65% of the nickel-cobalt-iron content.
29. A magnetic alloy comprising nickel between 9% and 81%, cobalt between 4% and 80% and iron between 5% and 45% of the entire nickel-cobalt-iron content.
30. A magnetic alloy comprising nickel between 15% and 81%, cobalt between 15% and 45% and iron between 9% and 45% of the entire nickel-cobalt-iron content characterized by a permeability which varies less than 5% over a range of flux densities from zero to 500 c. g. s. units.
31. A magnetic material comprising nickel, cobalt and iron in the approximate proportions of 60%, 15% and 25%, respectively.
32. A magnetic composition comprising nickel, cobalt and iron as essential elements thereof characterized in that it constitutes

at least part of a magnetic circuit for an electric circuit designed to operate by impressing upon the composition magnetizing forces of such magnitude as to produce 5 therein maximum flux densities of less than 1000 c. g. s. units.

33. A magnetic composition comprising nickel, cobalt and iron as essential elements thereof characterized in that over a range 10 of low magnetizing forces it has substantially constant permeability and that it forms part at least, of a magnetic circuit upon which are to be impressed a range of such 15 small magnetizing forces that the permeability remains substantially constant.

34. A magnetic composition comprising nickel, cobalt and iron as essential elements thereof characterized in that it constitutes 20 part at least of a magnetic circuit in inductive relation to a signaling conductor.

35. A magnetic composition comprising 25 nickel, cobalt and iron as essential elements thereof characterized in that it constitutes part at least of a magnetic circuit in inductive relation to a signaling conductor in a submarine cable.

36. A magnetic composition including 45% to 75% nickel and caused to have by the addition of suitable alloying elements and heat treatment an initial permeability 30 of 200 or more and a constancy of permeability within 5% up to a magnetizing force of at least .2 c. g. s. units.

37. A magnetic composition comprising 35 nickel and iron in the proportions of between 50% to 81% nickel and between 50% to 19% iron and caused to have by the addition of suitable alloying elements and heat treatment an initial permeability of at least 200 and constancy of permeability within 40 5% up to a magnetizing force of .2 c. g. s. units.

38. A magnetic material comprising 45 nickel, cobalt and iron as essential constituents thereof in which the nickel component comprises 50% to 65%, the cobalt component comprises 10% to 30% and the iron component comprises 10% to 30% of the nickel-cobalt-iron content.

In witness whereof, I hereunto subscribe 50 my name this 29th day of June, A. D. 1926.  
GUSTAF W. ELMEN.